# NEW EUROPEAN PATENT SPECIFICATION

(11) **EP 3 239 373 B2**
(45) Date of publication and mention of the opposition decision: **23.07.2025**
(45) Mention of the grant of the patent: 05.08.2020
(21) Application number: 16167320.7
(22) Date of filing: 27.04.2016
(51) Int. Cl.: D03D 1/00, D06M 16/00

(54) **A PROCESS OF PREPARING A DYED FABRIC INCLUDING A BACTERIAL BIOPOLYMER AND HAVING UNIQUE APPEARANCE**
VERFAHREN ZUR HERSTELLUNG EINES GEFÄRBTEN GEWEBES MIT EINEM BAKTERIELLEN BIOPOLYMER UND MIT EINZIGARTIGEM AUSSEHEN
PROCÉDÉ DE PRÉPARATION D'UN TISSU COLORÉ COMPRENANT UN BIOPOLYMÈRE BACTÉRIEN ET AYANT UNE APPARENCE UNIQUE

(43) Date of publication of application: 01.11.2017
(73) Proprietor: Sanko Tekstil Isletmeleri San. Ve Tic. A.S., 16400 Inegol - Bursa (TR)
(72) Inventor: ERYILMAZ, Jitka, 16400 Inegol - Bursa (TR); YUKSELEN, Onur, 16400 Inegol - Bursa (TR); COBANOGLU, Ozgur, 16400 Inegol - Bursa (TR)
(74) Representative: Gislon, Gabriele

(56) References cited:
- WO-A1-2008/020187
- DATABASE WPI Week 199802, Derwent World Patents Index; AN 1998-015342, XP002762770

## Description

### Field of the invention

The present invention relates to a process for the production of a fabric having a unique appearance, to a fabric obtained with said process and to clothing articles, i.e. garments, including said fabric. In particular, the present invention relates to a process for producing a woven fabric having a unique, e.g. "used" (i.e. worn-out) or "multi-shaded" appearance, wherein said process comprises the use of a biopolymer which is produced by a microorganism.

### Background of the invention

Worn out fabrics, especially denim, have enjoyed popularity in fashion industry due in particular to the finishing processes that can be applied to the fabric in order to create different appearances and thus different visible effects on the front side of the fabric, i.e. on the surface that is visible when the article made by the fabric is worn. In fact, the success in denim industry largely depends on creativity coming from a variety of fabric finishing processes that gives fabrics unique appearances.

The exterior appearance of a fabric, and thus of a clothing article made by the fabric, can be modified by using different finishing techniques.

JPH09279483 discloses a process wherein a fujiette fabric is treated with a culture medium for a cellulose-producing bacteria, and the cellulose-producing bacteria is cultured on the surface of the rayon filaments constituting the fabric until bacterial cellulose in the desired amount is produced.

A "used" or "vintage" or "worn-out" look of the fabric can be achieved by treating the fabric with a finishing process that is generally carried out on the garment or on the fabric. The known finishing processes may use specific chemicals, or mechanical abrasion, such as processes using stone-washing, acid wash, laser treatment and sandblasting. For example, in the stone washing, the fabric is washed in a cylinder in the presence of pumice stones.

While the wash cylinder rotates, the fabric is contacted by the stones that will remove part of the yarn fibers including the dye present on said fibers.

In this case, when a fabric and, in particular, an indigo dyed woven fabric is used, wherein the indigo dye is located on the surface of the yarns leaving the core of the yarns undyed, a stone wash (or sand blast) finishing process can be applied to allow varying amounts of the undyed cores of the indigo yarns to become visible.

These different finishing treatments result in different visible effects, in particular worn-out appearance, which make the fabric fashionable in the clothing and textile industries. However, the visible effects and appearance that are obtainable by the known finishing treatments, are limited. Therefore, garments made by different producers are often similar one to another, thus reducing the commercial desirability of the product and the possibility to distinguish a product from those of another producer.

A further disadvantage of traditional stone washing is that the stones can damage the fabric.

### Summary of the invention

It is an aim of the present invention to solve the above mentioned problems and to provide a process for the production of a fabric having a "unique" appearance; with "unique appearance" it is here meant an appearance different from the known ones, i.e. a look that was previously not attainable with known finishing processes, such as an improved "used" or "vintage" or "worn-out" appearance, in particular a distinctive worn-out appearance previously not obtainable with known processes.

Another aim of the present invention, is to provide a process for the production of a fabric having a "unique" appearance which is commercially desirable, recognizable and readily distinguishable from other products.

Still another aim of the present invention is to provide a process wherein damage to the yarns and the fabric made thereof is substantially avoided or is reduced, during the manufacturing and finishing processes. A further aim of the invention is to provide a finishing process that avoids or reduce the environmental costs of known finishing processes and that is less expensive than said processes.

These and other aims are achieved by a process according to claim 1.

In particular, the present invention refers to a process for producing a fabric, comprising the following steps:
a. Providing at least one plurality of warp yarns and at least one plurality of weft yarns;
b. Weaving said at least one plurality of warp yarns with said at least one plurality of weft yarns to provide a woven fabric, having a front side and a back side;
c. Providing at least a layer of at least one biopolymer which is produced by a microorganism on said yarns or on at least part of at least one side of said woven fabric to provide a composite fabric;
d. Dyeing at least part of said composite fabric, whereby at least part of the fabric yarns are dyed together with said biopolymer layer;
e. Removing at least part of said layer of biopolymer from said composite fabric to obtain a treated fabric.

Preferred embodiments are recited in the dependent claims.

In an exemplary embodiment, after step d. and before step e. the fabric is made, i.e. it is tailored, into a garment; the finishing processes may be applied to the fabric or to the garment including the fabric. In the following description reference will be made to the "fabric" to also identify a garment as far as at least the finishing processes are concerned, without limiting the scope of protection to treatment of the fabric only. As a matter of fact, the process of claim 1 may be carried out on a garment; claim 1 thus encompasses the treatment of a fabric in a garment.

By means of a process according to the invention, a "treated fabric", i.e. a woven fabric after finishing processes, with an improved (i.e. a "unique") aesthetical effect, can be obtained. The obtained fabric, i.e. the "treated" fabric, presents a "multi-shaded" effect, namely a "multi-shaded" appearance, previously not available through known finishing processes. Specifically, the obtained "multi-shaded" effect, is a distinctive appearance, preferably a "used" or "worn-out" appearance, which comprises a plurality of shades of color, which are distributed throughout the fabric (and, thus, throughout a garment comprising it) according to a non-reproducible distribution, such that the same distribution of shades cannot be reproduced from a fabric to another.

Without being bound to a specific scientific explanation, a possible explanation is that a biopolymer layer, being produced by living microorganisms, may not be structurally identical to another biopolymer layer, even if it has been produced by the same microorganisms and in the same conditions. Therefore, it has been observed that two different biopolymer layers provide for two different dyeing-results of the biopolymer layers themselves and of the fabrics (or yarns) coupled therewith, as well.

As above mentioned, by means of a process according to the invention a "treated fabric", i.e. a woven fabric after finishing processes, with a "unique" aesthetical effect, can be obtained; in other words, two woven fabrics that are "treated" with the process of the invention, show two different aesthetical results, i.e. the same distribution of color shades is not reproduced from a fabric to another. Thus, each "treated fabric", obtained by the process of the invention, shows an aesthetical appearance that is substantially "unique", i.e. an aesthetical appearance that is substantially "not reproducible".

The treated fabric of the invention, as obtained after the removal of at least part of the biopolymer layer from the dyed composite fabric, shows a plurality of color shades, according to the amount of dye which has been absorbed by the biopolymer layer and reached the underlying woven fabric.

This is particularly true when, according to a preferred embodiment, said at least one biopolymer layer has a thickness "T" that is non-uniform throughout the extension of the biopolymer layer, i.e. that is not the same throughout the whole extension of the biopolymer layer.

In fact, without being bound to a specific scientific explanation, it has been observed that the dye uptake of the fabric provided with the claimed biopolymer layer as obtained in step c. of the process of the invention, is variable in relationship with the variable thickness of the biopolymer layer.

In particular, it has been observed that, the higher is the thickness T, the higher is the dye uptake of the layer of biopolymer, i.e., the amount of dye which is absorbed by the biopolymer layer, and the less is the amount of dye that arrives to the yarns and that dyes the yarns provided with the biopolymer layer. In other words, when, for example, a composite fabric comprises a biopolymer layer having non-uniform (i.e. "variable") thickness, different amounts of dye reach the underlying surface (for example, the front side) of the woven fabric, according to the thickness of the biopolymer layer so that the fabric yarns take on different amounts of dye in different regions.

It has to be noted that the thickness ("T") of the biopolymer layer of a composite fabric according to the invention and the amount of the dye which reaches the woven fabric provided with the biopolymer layer are inversely proportional. In other words, the higher is the thickness of the biopolymer layer, the lower is the amount of dye that reaches the woven fabric provided with the biopolymer layer. For example, if the thickness of the biopolymer layer of a composite fabric according to the invention is high, a high amount of dye is absorbed by the biopolymer layer and only a low amount of dye (or none) reaches the woven fabric provided with the biopolymer layer. Therefore, after the removal of the biopolymer layer, a treated fabric that is slightly colored (i.e. that is a colored in a light shade of color) or that is substantially non-colored is obtained. On the contrary, for example, if the thickness "T" of the biopolymer layer is low, a low amount of dye is absorbed by the biopolymer layer, and thus a high amount of dye reaches the surface (i.e., for example, the front side) of the woven fabric provided with the biopolymer layer. Therefore, after the removal of the biopolymer layer, a treated fabric that is intensely colored (i.e. that is colored in a dark shade of color) is obtained.

As used herein, the term "thickness", refers to the distance between the top and bottom or front and back surfaces of something; e.g., the distance between the top and bottom surfaces of the biopolymer layer. The bottom surface of the biopolymer layer is the surface of the biopolymer layer which contacts the fabric or yarns. The top surface of the biopolymer layer is the surface of the biopolymer layer, opposite to the bottom surface, which does not contact the fabric or yarns.

As used herein, the term "uniform thickness", refers to a thickness that is substantially constant (substantially non-variable); e.g. the distance between the top and bottom surfaces of the biopolymer layer does not substantially change along the extension of the biopolymer layer.

On the contrary, as used herein, the term "non-uniform thickness", refers to a thickness that is variable; e.g. the distance between the top and bottom surfaces of the biopolymer layer varies (i.e. "changes", i.e. it is not constant) along the extension of the biopolymer layer.

According to preferred embodiments, at least part of said biopolymer layer is a discontinuous layer.

For example, a biopolymer layer can be a discontinuous biopolymer layer, i.e. a biopolymer layer can presents interruptions along its extension. In this case, for example, a fabric or a yarn that is provided with a discontinuous biopolymer layer presents regions on its surface (e.g. the front side of a woven fabric) that are not "covered" by the biopolymer layer.

Advantageously, considering, for example, a composite fabric (as obtainable in step c. of the process of the invention) wherein the biopolymer layer is discontinuous, i.e. wherein the biopolymer layer presents interruptions throughout its extension, regions of the woven fabric provided with biopolymer layer, result to be "not-covered" by the biopolymer layer. Therefore, when the composite fabric is dyed according to step d. of the process of the invention, regions of the woven fabric that are "not-covered" by the biopolymer layer are completely and "directly" dyed; in other words where the woven fabric is not "covered" by the biopolymer layer, the dye is applied directly on the woven fabric.

Advantageously, when a composite fabric comprises a discontinuous biopolymer layer, a treated fabric having a patterned multi-shaded effect can be obtained.

In other words, a discontinuous biopolymer layer according to the invention can present a predetermined "patterned" distribution of "interruptions" in order to provide a treated fabric with a predetermined pattern of regions of the woven fabric that are "completely" and "directly" dyed, as above mentioned. Therefore, once the biopolymer layer is removed according to step e. of the process of the invention, a treated fabric having a multi-shaded effect further comprising a patterned distribution of "completely dyed" regions can be obtained. On the contrary, where the woven fabric is provided with the biopolymer layer, once the biopolymer layer is removed after the dyeing, regions having multi-shaded effect, as above defined, are obtained. In other words, the biopolymer layer can act as a "stencil" when the composite fabric is dyed.

According to embodiments of the invention, variation within the weaving pattern of the woven fabric provides further visual effects. In fact, it has been observed that the weaving pattern contributes to the final appearance.

According to a preferred embodiment, the biopolymer layer is a non-uniform discontinuous layer. In other words, a bacterial biopolymer according to the invention can have a variable thickness and interruptions throughout its whole extension.

According to embodiments of the invention, the woven fabric is provided with at least one biopolymer layer on at least the front side and/or the back side.

As used herein, the term "front side" of the fabric, refers to the side of the fabric which is the external visible side when a garment comprising the fabric is worn. As used herein, the term "back side" of the fabric, refers to the side of the fabric which is the internal not visible side when a garment comprising the fabric is worn.

According to embodiments, the woven fabric is provided with at least one biopolymer layer on both the front side and the back side.

For example, a woven fabric according to the invention can be provided with two biopolymer layers, namely with a first biopolymer layer on its front side and with a second biopolymer layer on its back side, thus providing a composite fabric comprising a woven fabric and two biopolymer layers.

According to exemplary embodiments, the first biopolymer layer (on the front side) and the second biopolymer layer (on the back side) can comprise the same or a different bacterial biopolymer.

As used herein, the terms "bacterial biopolymer layer", "bacterial polymer layer", "biopolymer layer" and "polymer layer" refer to a layer comprising at least one bacterial biopolymer.

As used herein, the terms "bacterial biopolymer" and "bacterial polymer" refers to all the polymers the can be produced by a microorganism, where the term "microorganism" encompasses not genetically modified (i.e. wild type) microorganisms and genetically modified microorganism. For example, a microorganism can be genetically modified in order to produce a bacterial biopolymer which is not produced by the same microorganism when it is not genetically modified (i.e., when it is a wild type microorganism).

As used herein, the term "microorganism" refers to small unicellular or multicellular living organisms that are too small to be seen with naked eye but are visible under a microscope, and encompasses bacteria, yeast, fungi, viruses and algae. As above mentioned, the term "microorganism" encompasses not genetically modified (i.e. wild type) microorganisms and genetically modified microorganism as well.

In the present description, reference is made to "bacterial biopolymer" for sake of simplicity, without however limiting the scope of the invention to polymers produced by "bacteria" only, but encompassing all the polymers that can be produced by a microorganism as above defined.

According to embodiments of the invention, the biopolymer layer comprises a sugar-based biopolymer or an amino acid-based biopolymer or a mixture thereof.

As used in the present description, the term "sugar-based biopolymer" encompasses linear and branched polysaccharides, variants and derivatives thereof. An exemplary sugar-based biopolymer is cellulose.

As used in the present description, the term "amino-acid based biopolymer" encompasses linear and branched polypeptides, variants and derivatives thereof. An exemplary amino acid-based biopolymer is collagen.

According to a preferred embodiment, said bacterial biopolymer is selected from bacterial cellulose, bacterial collagen or mixtures thereof.

According to preferred embodiments of the invention, said biopolymer layer comprises a bacterial biopolymer selected from cellulose, collagen, cellulose/chitin copolymer, silk, and mixtures thereof. These biopolymers are known per se in the art.

A biopolymer layer according to the invention (e.g., cellulose) is produced by culturing biopolymer-producing microorganisms, preferably selected from bacteria, algae, yeast, fungi and mixtures thereof.

For example, a layer of bacterial collagen can be provided to the front side of the woven fabric and a layer of bacterial cellulose can be provided to the back side of the woven fabric.

According to embodiments of the invention, biopolymer-producing bacteria are selected from *Gluconacetobacter, Aerobacter, Acetobacter, Achromobacter, Agrobacterium, Azotobacter, Salmonella, Alcaligenes, Pseudomonas; Rhizobium, Sarcina, Streptoccoccus* and *Bacillus* genus, and mixtures thereof. According to embodiments of the invention, biopolymer-producing algae are selected from *Phaeophyta, Rhodophyta* and *Chrysophyta,* and mixture thereof.

For example, bacterial cellulose can be produced by culturing strains of Acetobacter bacteria, such as strains of *Acetobacter xylinum,* and/or by culturing strains of Gluconacetobacter, such as strains of *Gluconacetobacter hansenii.*

For example, bacterial collagen can be produced by culturing bacterial strains of Bacillus, *Pseudomonas, Streptoccoccus* or bacterial strains which have been genetically modified to obtain modified strains that produce collagen. Advantageously, bacterial collagen can be produced on the fabric to provide an artificial leather-like material, ("artificial leather" or "artificial skin", wherein the main structural component of "leather" and "skin" is type I collagen in the form of strong fibrils). For example, bacterial cellulose/chitin copolymer can be produced by culturing strains of *Acetobacter xylinum* which have been genetically modified to obtain modified strains that produce bacterial cellulose/chitin copolymer.

According to exemplary embodiments of the invention, the biopolymer producing microorganisms are a mixture of wild type and genetically modified microorganisms.

According to the embodiment, step c. of the process of the invention is carried out by contacting at least part of at least one plurality of warp yarns and/or at least part of at least one plurality of weft yarns, or at least part of a woven fabric with a culture of biopolymer-producing microorganisms, and culturing said biopolymer-producing microorganisms, to provide at least part of said at least one plurality of warp yarns and/or at least part of said at least one plurality of weft yarns, or at least part of said woven fabric with a biopolymer layer.

In other words, a composite fabric according to step c. of the present invention is obtained by providing a woven fabric with a biopolymer layer, that is "grown" (i.e. produced) directly on the fabric.

For example, a composite fabric according to the invention, is advantageously obtained by contacting the front side and/or the back side of a woven fabric, with a culture of biopolymer-producing microorganisms, and culturing said biopolymer-producing microorganisms. More in detail, once the woven fabric is contacted with a culture of biopolymer-producing microorganisms, biopolymer-producing microorganisms are cultured, to produce a layer of biopolymer directly on the fabric, thus providing a composite fabric according to step c. of the process of the invention.

According to embodiments, at least part of at least one plurality of warp yarns and/or at least part of at least one plurality of weft yarns, as provided in step a. of the process of the invention, are provided with a biopolymer layer before the weaving according to step b.

For example, a biopolymer layer (e.g. a cellulose layer), preferably a thin biopolymer layer(e.g. a "film" of biopolymer) can be grown directly on cotton yarns.

Advantageously, a biopolymer layer, provided onto yarns (warp and/or weft yarns) before the weaving, act as sizing agent, thus protecting the yarns during the weaving process.

Additionally, the biopolymer layer provided onto the yarns protects the yarns from damages also after the weaving step.

Moreover, when the biopolymer layer (e.g. a biopolymer film) is grown (i.e. produced) directly on the warp and/or weft yarns, it is possible to skip the step of sizing the yarns before the weaving and to skip the step of de-sizing after the weaving, thus reducing the costs for the production.

According to exemplary embodiments, at least part of at least one plurality of warp yarns and/or at least part of at least one plurality of weft yarns, as provided in step a. of the process of the invention, are provided with a biopolymer layer and dyed before the weaving step according to step b.

For example, a biopolymer layer according to the invention can be produced (i.e. "grown") on the yarns by contacting said yarns, with a culture of biopolymer-producing microorganisms, and culturing said biopolymer-producing microorganisms, before the weaving, thus providing "composite yarns".

According to embodiments of the invention, the "composite yarns" may be woven to provide a woven fabric provided with a biopolymer layer, which may be subsequently dyed. Alternatively, or additionally, the composite yarns may be dyed before the weaving step.

According to embodiments, a biopolymer layer is provided to a woven fabric according to step c. by growing, i.e. producing, the biopolymer layer on the fabric.

According to the embodiment, step c. of the process of the invention is carried out by contacting at least part of the woven fabric (or at least some of the yarns before weaving) with a culture of biopolymer-producing microorganisms, and culturing said biopolymer-producing microorganisms, to provide the woven fabric with a biopolymer layer, thus obtaining a composite fabric.

Advantageously, by producing (i.e. growing) the biopolymer layer on the woven fabric (or on at least some of the yarns before weaving), a non-uniform biopolymer layer, as above discussed, is obtained.

According to exemplary embodiments, the woven fabric (or the yarns before the weaving) may be contacted with a culture of biopolymer-producing microorganisms, by dipping the fabric (or the yarns) into the culture of biopolymer-producing microorganisms.

In other words, according to exemplary embodiments, at least part of the woven fabric, or at least part of the yarns (e.g. the yarns before the weaving) is contacted with a culture of microorganisms producing a bacterial biopolymer, by dipping said at least part of said woven fabric or at least part of said yarns into said culture of biopolymer-producing microorganisms.

Advantageously, when the woven fabric is dipped into the culture of biopolymer-producing microorganisms, the biopolymer layer grows on both the sides (i.e. the front side and the back side of the woven fabric), thus providing a composite fabric wherein the woven fabric is provided with two biopolymer layers, which comprise the same biopolymer.

According to other exemplary embodiments, the culture of biopolymer-producing microorganisms is sprayed on at least part of said woven fabric (or on at least some of the yarns before weaving), preferably on at least part of the front side of said woven fabric.

According to embodiments, the culture of biopolymer-producing microorganisms is sprayed on at least part of said woven fabric through a mesh wire.

Advantageously, by spraying the culture of biopolymer-producing microorganisms on at least part of said woven fabric through a mesh wire, the biopolymer layer is grown, i.e. produced, on the woven fabric as a discontinuous and non-uniform biopolymer layer, as above discussed.

Preferably, the mesh wire is removed before dyeing once the bacterial biopolymer is grown on the woven fabric. Advantageously, when the mesh wire is removed after the bacterial biopolymer is grown on the woven fabric, a biopolymer layer having a defined pattern is obtained.

According to a preferred embodiment of the invention, the warp yarns and/or weft yarns are hydrophilic yarns.

Advantageously, when the warp yarns and/or the weft yarns are hydrophilic yarns, the culture medium of the biopolymer-producing microorganisms is absorbed by the yarns (before the weaving) or by the woven fabric, thus providing nutrients to the microorganisms and ingredients for the synthesis of the biopolymer layer, directly on the woven fabric.

According to embodiments of the invention, hydrophilic yarns are natural yarns, i.e. yarns that are made of natural fibers.

Preferably, natural yarns comprise natural fibers selected from cotton, wool, flax, kenaf, ramie, hemp, and mixtures thereof.

According to embodiments of the invention, hydrophilic yarns are synthetic yarns, i.e. yarns that are made of synthetic fibers.

Preferably, synthetic yarns comprise synthetic fibers selected from polyester, rayon, nylon, lycra and mixtures thereof. According to a preferred embodiment, synthetic yarns and/or synthetic fibers are treated (i.e. finished) in order to provide synthetic yarns and/or synthetic fiber having hydrophilic properties.

For example, a synthetic yarns and/or synthetic fibers, that is not hydrophilic per se, can be treated with a hydrophilizing agent in order to gain hydrophilic features. According to embodiments, hydrophilic yarns are mixed yarns, i.e. yarns that comprise both natural and synthetic fibers. In this case, for example, a hydrophilic mixed yarn can be obtained by mixing hydrophilic natural fibers and hydrophobic synthetic fibers.

In embodiments of the invention, the warp yarns and/or the weft yarns are selected from natural yarns, synthetic yarns and mixed yarns. According to a preferred embodiment, warp yarns and/or weft yarns are natural yarns. Preferably, natural yarns comprise natural fibers selected from cotton, wool, flax, kenaf, ramie, hemp, and mixtures thereof.

In other embodiments of the invention, the warp yarns and/or the weft yarns are synthetic yarns, preferably thermoplastic yarns, more preferably thermoplastic elastomeric yarns. Preferably, synthetic yarns comprise synthetic fibers selected from polyester, rayon, nylon, lycra and mixtures thereof.

In exemplary embodiments of the invention, the warp yarns and/or the weft yarns of the woven fabric are mixed yarns, i.e. yarns comprising both natural fibers and synthetic fibers. In exemplary embodiments of the invention, natural fibers and yarns are hard fibers and yarns. In exemplary embodiments of the invention, synthetic fibers and yarns are elastomeric fibers and yarns.

Suitable elastomeric yarns are yarns containing elastomeric fibers. An "elastomeric fiber" is a fiber made of a continuous filament or a plurality of filaments which have an elongation at break of at least 100%, independent of any crimp. Break elongation may be measured e.g. according to ASTM D2256/D2256M-10(2015). An "elastomeric fiber" is a fiber that after being stretched to twice its length and held for one minute at said length, will retract to less than 1,5 times its original length within one minute of being released. According to a preferred embodiment, a woven fabric suitable for use in the invention comprises warp yarns and weft yarns woven together, and has a front side and a back side, wherein said warp yarns and at least one plurality of weft yarns form a base layer of said woven fabric, and wherein a plurality of warp yarns and/or at least one plurality of weft yarns forms an additional layer of loop portions, on at least one of the sides of said woven fabric.

According to exemplary embodiments, fabric structures suitable to be used as "woven fabric" in a process according to the present invention are disclosed in patent application US2015/0038042 (see in particular paragraphs [0013], [0019]-[0027], [0030], [0031], [0033], [0049]-[0051], [0054], [0055], [0060], [0066], [0068]-[0071], [0075], [0076], [0078]-[0083], [0086], [0089]-[0117]) and in patent application US2013/0048140 (see in particular paragraphs [0007], [0010], [0013]-[0018], [0041]-[0046], [0048]-[0050], [0054]-[0059] and Examples 1, 3-8 and 10) whose descriptions are incorporated herein by reference.

In a preferred embodiment, at least part of said additional layer of loop portions is included, e.g. embedded, into the biopolymer layer. According to exemplary embodiments, the composite fabric of the present invention, may be a composite fabric as disclosed in co-pending application having title "Composite fabric comprising a bacterial biopolymer layer" in the name of the present applicant.

According to preferred embodiments, the woven fabric is a denim fabric.

According to embodiments of the invention, the step d. of the process of the invention is carried out by print-dyeing, preferably indigo print-dyeing, or by dipping the composite fabric into a dye bath (preferably, an indigo bath).

The best results are obtained with print-dyeing, dye-coating where the dye is applied only on the side of the fabric where the bacterial biopolymer (e.g. cellulose) is grown. That way the bacterial biopolymer (e.g. cellulose) behave as a barrier, hence unique visual effects can be obtained. However, very good results were also obtained via conventional indigo dyeing methods, where the fabric is dipped into indigo bath (both sides of the fabric are dyed) and only during the washing treatments, as the bacterial biopolymer (e.g. cellulose) is removed, the color-shade variation appears. Here again, the thickness of the bacterial cellulose has an important role. The thicker the biopolymer layer (e.g. cellulose) is, the less of the dye can penetrate to the center of individual fibers, hence a shallow ring effect is observed and vice versa when the thickness is less the ring effect is deeper. This overall, creates visual color variations especially during washing treatments.

Preferably, when the composite fabric, as obtained in step c., is dyed by print-dyeing, the print-dyeing is carried out on the side of the composite fabric where the biopolymer layer is placed.

In this case, advantageously, the biopolymer layer acts as a barrier during the print-dyeing process, thus preventing damages to the woven fabric underlying the biopolymer layer, and preventing the penetration of a great amount of dye into the woven fabric. For example, as above discussed, depending on the thickness and/or the pattern (i.e. continuity or discontinuity) of the biopolymer layer, the amount of dye which reaches and penetrates into the woven fabric varies.

According to embodiments, step d. is carried out by dyeing said composite fabric with a dye selected from the group of indigo dye, sulphur dye, pigment dye, reactive dye. The preferred way of application of these-lected dye is print-dyeing; when print dyeing is used, any dye such as vat, direct, reactive can be used.

According to exemplary embodiments, step e. of the process of the invention is carried out by finishing treatments, e.g. rinse wash, enzyme washing, stone washing, laser treatments etc., as well as laundry washing, in order to remove at least part of said at least one biopolymer layer from said composite fabric, thus providing a treated fabric according to the invention.

In other words, a biopolymer layer can be removed, at least in part, from the composite fabric by washing, e.g. laundry washing, the dyed composite fabric with water, thus substantially avoiding the use of chemical agents. According to embodiments, the step e. of the process of the invention is carried out by abrading at least part of said at least one biopolymer layer from said composite fabric.

In other words, the removal of the biopolymer layer from the composite fabric, to obtain a treated fabric is carried out by abrading (i.e. "rubbing", "scraping") the biopolymer layer, damaging the biopolymer layer, removing substantially all the biopolymer layer, without damaging the fabric.

According to a preferred embodiment, step e. is carried out by stone-washing said dyed composite fabric obtained in step d.

Advantageously, the stone washing of the composite fabric as obtained in step d. of the process of the invention, i.e. the washing of the composite fabric in the presence of pumice stones, allows the effective and fast removal of the biopolymer layer, without damaging the woven fabric underlying the biopolymer layer, thus providing a treated fabric having a multi-shaded effect without affecting (i.e. reducing) the mechanical integrity and the properties of the fabric, such as the tensile strength.

According to a preferred embodiment, step e. is carried out by bio-stoning said dyed composite fabric obtained in step d.

Advantageously, the bio-stoning ofthe composite fabric as obtained in step d. of the process of the invention, i.e. the washing of the composite fabric in the presence of enzymes able to provide the removal of the biopolymer layer from the composite fabric, provides a treated fabric having a multi-shaded effect without affecting (i.e. reducing) the mechanical integrity and the properties of the fabric, such as the tensile strength, and substantially avoiding the use chemical agents and pollutants.

According to embodiments of the invention, step e. is carried out by laundry washing and/or stone washing and/or bio-stoning a garment comprising a composite fabric as obtainable in step d. of the process of the invention. According to embodiments of the invention, step e. is carried out by laser treatment.

Another object of the invention is a treated fabric as obtained by a process according to the invention.

Advantageously, a treated fabric obtained through the process of the invention presents a "multi-shaded" effect, namely a "multi-shaded" appearance, previously not available through known finishing processes. Specifically, as above discussed, the obtained "multi-shaded" effect comprises a plurality of shades of color, which are distributed throughout the fabric (and throughout a garment comprising it) according to a non-reproducible pattern, such as the same distribution of shades cannot be reproduced from a fabric to another.

According to an aspect of the invention, the "multi-shaded" effect of the treated fabric, depends on the thickness and/or the pattern (i.e. the continuity or discontinuity) of the biopolymer layer, which is provided onto the non-treated woven fabric, according to point c. of the process of the invention. For example, a "non-treated" woven fabric is provided with a biopolymer layer, thus providing a composite fabric. The composite fabric is subsequently dyed. At least part of the biopolymer layer is then removed from the dyed composite fabric, thus providing a treated fabric having a "multi-shaded" effect.

As above mentioned, the "multi-shaded" effect of the treated fabric, depends of the thickness and/or the pattern (i.e. the continuity or discontinuity) of the biopolymer layer.

For example, a biopolymer layer can have a thickness T which schematically assumes three different values, namely T1, T2 and T3, where T3>T2>T1.

In this case, the dye uptake of the biopolymer layer where the thickness is T3 is more than the uptake where the thickness is T2, which is, in turn, more than the uptake where the thickness is T1. Therefore, if a certain amount of dye reaches the woven fabric underlying the biopolymer layer where the thickness of the biopolymer layer is T1, a lower amount of dye reaches the woven fabric where the thickness of the biopolymer layer is T2, and an even lower amount of dye reaches the woven fabric where the thickness is T3. In this case, a treated fabric having three different shades of color can be obtained.

It has to be noted that the above mentioned example is merely a schematic description, in fact, the treated fabric of the invention has a "multi-shaded" appearance, i.e. the treated fabric presents numerous different color shades, due to the different penetration of the dye throughout the biopolymer layer.

According to embodiments of the invention, a treated fabric according to the invention comprises dyed yarns and portions of a dyed biopolymer layer; in other words, in embodiments of the invention a treated fabric as obtained by a process according to the invention comprises residual bacterial biopolymer regions, i.e. regions wherein the biopolymer layer has been not completely removed.

A further object of the present invention is a garment comprising a treated fabric as obtained by the process of the invention.

According to a preferred embodiment, in a garment according to the invention, the front side of the treated fabric is the external visible side when the garment is worn, and the back side of the treated fabric is the internal not visible side when the garment is worn.

Another object of the present invention is a garment comprising a composite fabric as obtained with the process of the invention. Preferably, the fabric is tailored into a garment after step b. or c. of the process of the invention.

According to embodiments of the invention, when a garment comprises a composite fabric as obtained in step c. or step d. of the process of the invention, a "multi-shaded" effect can be advantageously obtained by removing at least part of the biopolymer layer from the garment, i.e. by removing at least part of the biopolymer layer from the composite fabric, after the composite fabric has been used for the production of a garment.

### Brief description of the drawings

Further aspects and advantages of the present invention will be discussed more in detail with reference to the enclosed drawings, given by way of nonlimiting example, wherein:
- Figure 1 is a perspective view of a portion of an exemplary woven fabric according to the invention, before undergoing step c. of the process of the invention, i.e. a not-treated woven fabric;
- Figure 2 is a perspective view of a portion of a composite woven fabric according to the invention, as obtainable after step c. of the process of the invention, i.e. a woven fabric provided with a polymer layer;
- Figure 3 is a perspective view of a portion of an exemplary composite fabric according to the invention, as obtainable after step d. of the process of the invention, i.e. a dyed composite fabric;
- Figures 4, 5, 6 and 7 are perspective views of exemplary embodiments of the treated fabric as obtainable by the process of the invention;
- Figure 8 shows an embodiment of the invention, wherein a culture of biopolymer-producing microorganisms is sprayed on an exemplary woven fabric through a mesh wire;
- Figure 9 is a perspective view of a portion of an exemplary composite fabric according to the invention, having a discontinuous biopolymer layer;
- Figure 10 is a perspective view of a portion of an exemplary composite fabric according to the invention, having a discontinuous biopolymer layer, after the dyeing process;
- Figure 11 is a perspective view of an exemplary embodiment of the treated fabric as obtainable by the process of the invention.

### Detailed description of the invention

According to an aspect of the invention, the structure of the treated fabric is substantially the same of the non-treated woven fabric (i.e. the woven fabric before steps c., d. and e. of the process of the invention); in other words, the process of the invention does not substantially modify the structure of the woven fabric which is subjected to the process of the invention.

Therefore, in this embodiment the "woven fabric" 1 (i.e. the fabric before steps c., d. and e. of the process of the invention) and the "treated fabric" 100 (i.e., the fabric after step e. of the process of the invention) shall be interpreted to be the same fabric before and after the process of the invention. In other words, a treated fabric is the woven fabric after having been treated according to the invention.

Figure 1 is a perspective view of a portion of an exemplary woven fabric 1 according to the invention, before undergoing step c. of the process of the invention, i.e. a not-treated woven fabric.

Figure 1 shows a woven fabric 1, having warp yarns 2 and weft yarns 3, and having a front side 5 and a back side 6. Weft yarns 3 and warp yarns 2 are woven in a pattern wherein weft yarns 3 pass over two warp yarns 2, on the front side 5 of the fabric, and under one warp yarn 2 on the back side 6.

It has to be noted that the weaving pattern illustrated in the present figures have to be intended as merely representative, and not limiting of the scope of the invention; in fact any kind of weaving pattern have to be considered as included in the scope of the claims. As above mentioned, the weaving pattern may contribute to the final appearance.

The woven fabric 1 represented in Figure 1 is not dyed.

Figure 2 is a perspective view of a portion of an exemplary composite fabric 10, as obtainable after step c. of the process of the invention. A woven fabric 1 is provided with a biopolymer layer 4, on its front side 5, thus providing a composite fabric 10.

The back side 6 of the woven fabric 1 is also indicated in Figure 2. In this case, the back side 6 of the woven fabric 1 corresponds to the back side of the composite fabric 10.

In the embodiment of Figure 2, the biopolymer layer 4 is schematically represented as a continuous and uniform layer, i.e. a layer that covers continuously (i.e. without interruptions) the front side 5 of the woven fabric 1 and that maintains substantially the same thickness T over its entire extension.

According to a preferred embodiment of the invention, the biopolymer layer 4 is produced directly on the woven fabric 1, namely by culturing biopolymer-producing microorganisms directly on the woven fabric 1.

For example, the woven fabric 1 is contacted with a culture of biopolymer-producing microorganisms, which are cultured directly on the woven fabric 1. By culturing the microorganisms directly on the woven fabric 1, the growing (i.e. the production) of a biopolymer layer 4 on the woven fabric 1 is obtained.

In embodiments of the invention, the biopolymer layer 4 is a non-uniform layer, i.e. it has a thickness T which is variable throughout the extension of the biopolymer layer 4.

In embodiments of the invention, the biopolymer layer 4 is a discontinuous layer, i.e. is an interrupted layer, thus providing areas of the woven fabric 1 which are not provided (i.e. not covered) with the biopolymer layer 4.

Figure 3 is a perspective view of a portion of an exemplary composite fabric 10, as obtainable after step d. of the process of the invention, i.e. a dyed composite fabric. Figure 3 shows, in particular, the biopolymer layer 4 after dyeing. Similarly to Figure 2, the biopolymer layer 4 is schematically represented as a continuous and uniform layer, i.e a layer that covers continuously (i.e. without interruptions) the front side 5 of the woven fabric 1 and that maintains substantially the same thickness T over its entire extension.

However, as above mentioned, in embodiments of the invention the biopolymer layer 4 is discontinuous and/or non-uniform. The back side 6 of the woven fabric 1 is also indicated in Figure 3. In this case, the back side 6 of the woven fabric 1 corresponds to the back side of the composite fabric 10.

Figure 4 shows a perspective view of an exemplary embodiment of a treated fabric 100 as obtainable by the process of the invention, i.e. after that at least part of the biopolymer layer 4 is removed from the composite fabric 10.

Figure 4 shows a treated fabric 100, having warp yarns 2 and weft yarns 3, and having a front side 5 and a back side 6. Weft yarns 3 and warp yarns 2 are woven in a pattern wherein weft yarns 3 pass over two warp yarns 2, on the front side 5 of the fabric, and under one warp yarn 2 on the back side.

Figure 4 shows, schematically, an embodiment wherein the biopolymer layer 4 has been completely removed from the composite fabric 10, e.g. from the front side 5 of the woven fabric 1.

The treated fabric 100, in the embodiment represented in Figure 4, presents, on its front side 5, first regions 7 that are intensely colored, second regions 8 that are slightly colored (i.e., dyed with a lighter shade of color than the first regions 7), and third regions 9 that are substantially not colored, i.e. not dyed. Figure 4 shows an embodiment if the treated fabric 100 wherein first regions 7 cover the most of the front side 5 of the treated fabric 100. The treated fabric 100 of Figure 4 presents second regions 8 which are colored with a lighter shade of color than the first regions 7, and also presents third regions 9 which are substantially not dyed.

Accordingly, a treated fabric 100 as shown in Figure 4 is substantially intensely dyed, and presents regions in a lighter shade and not-dyed regions, thus providing a substantially "light on dark" shade effect, namely a "light on dark" worn out look.

It has to be noted that Figure 4 is merely a schematic representation of a treated fabric 100 according to the invention; in fact, the treated fabric 100 of the invention have a "multi-shaded" appearance, i.e. the treated fabric 100 presents numerous different color shades, due to the different penetration of the dye throughout the biopolymer layer 4, namely through the thickness T of the biopolymer layer 4.

This is particularly true in the embodiments of the invention, where the biopolymer layer 4 has a thickness T that is non-uniform, i.e. that is not the same throughout the extension of the biopolymer layer 4; in other words, where thickness T assumes different values in different regions of the biopolymer layer 4.

In fact, if the composite fabric 10 presents a biopolymer layer 4 having variable thickness T, the dye uptake of the composite fabric 10 is variable in relationship with the variable thickness T of the biopolymer layer 4.

In particular, it has been observed that, the higher is the thickness T, the higher is the dye uptake of the biopolymer layer 4. In other words, when a composite fabric 10 presents a biopolymer layer 4 having variable thickness T, different amounts of dye reach the surface (i.e., for example, the front side 5) of the woven fabric 1, in relationship with the variation of the thickness T along the extension of the biopolymer layer 4.

For example, if the thickness T of the biopolymer layer is high, only a little amount (or none) dye reaches the surface (i.e., for example, the front side 5) of the woven fabric 1, thus providing a treated fabric 100 with second regions 8 that are slightly colored and/or third regions 9 that are substantially not colored, i.e. not dyed.

On the contrary, for example, if the thickness T of the biopolymer layer is low, a greater amount of dye reaches the surface (i.e., for example, the front side 5) of the woven fabric 1, thus providing a treated fabric 100 with first regions 7, that are intensely colored.

According to preferred embodiments of the invention, growing the biopolymer layer 4 directly on the woven fabric 1, a biopolymer layer 4 having a variable thickness T can be obtained.

For example, a treated fabric 100, according to Figure 4, can be obtained when the biopolymer layer 4 (removed according to step e. of the process of the invention) has a thickness T having value T1 in correspondence of the first regions 7, a thickness T2>T1 in correspondence of second regions 8, and a thickness T3>T2>T1 in correspondence of third regions 9. In this case, according to Figure 4, where the thickness T of the biopolymer layer 4 is T3, substantially all the dye is absorbed by the biopolymer layer 4; in other words, the dye does not substantially reach the surface (e.g. the front side 5) of the woven fabric 1, thus providing a treated fabric 100 having third regions 9 that are substantially not colored. Additionally, where the thickness T of the biopolymer layer 4 is T2, only part of the dye reaches the surface (e.g. the front side 5) of the woven fabric 1, thus providing a treated fabric 100 having second regions 8 that are slightly colored. Moreover, where the thickness T of the biopolymer layer 4 is T1, substantially all the dye reaches the surface (i.e. the front side 5) of the woven fabric 1, thus providing a treated fabric 100 having first regions 7, that are intensely colored.

Accordingly, a treated fabric 100 as shown in Figure 4 is substantially dyed, and presents not-dyed regions (namely third regions 9), and regions colored in a lighter shade (namely second regions 8), thus providing a "light on dark" shade effect, namely a "light on dark" worn out look.

Figure 5 shows a perspective view of an exemplary embodiment of a treated fabric 100 as obtainable by the process of the invention, i.e. after that at least part of the biopolymer layer 4 is removed from the composite fabric 10.

Figure 5 shows a treated fabric 100, having warp yarns 2 and weft yarns 3, and having a front side 5 and a back side 6. Weft yarns 3 and warp yarns 2 are woven in a pattern wherein weft yarns 3 pass over two warp yarns 2, on the front side 5 of the fabric, and under one warp yarn 2 on the back side 6.

Figure 5 shows an embodiment, wherein the biopolymer layer 4 has been completely removed the composite fabric 10, e.g. from the front side 5 of the woven fabric 1, in step e. of the process of the invention.

Figure 5 represents a treated fabric 100 having, in its front side 5, first regions 7 that are intensely colored, second regions 8 that are slightly colored (i.e., dyed with a lighter shade of color than the first regions 7), and third regions 9 that are substantially not colored, i.e. not dyed. Figure 5 shows an embodiment of the treated fabric 100 wherein third regions 9 cover the most of the front side 5 of the treated fabric 100. Treated fabric 100 presents first regions 7, which are intensely dyed, and second regions 8 which are colored with a lighter shade of dye than the first regions 7.

Therefore, a treated fabric 100 as shown in Figure 5 is substantially not dyed, and presents intensely dyed regions (namely first regions 7), and slightly colored regions (namely second regions 8), thus providing a "dark on light" shade effect, namely a "dark on light" worn out look.

For example, a treated fabric 100 according to Figure 5 can be obtained, when the biopolymer layer 4 (removed with step e. of the process of the invention) has a thickness T1 in correspondence of the first regions 7, a thickness T2>T1 in correspondence of second regions 8, and a thickness T3>T2>T1 in correspondence of third regions 9.

For example, a biopolymer layer 4 having variable thickness T can be obtained by growing (i.e. producing) said biopolymer directly on the surface of the fabric, namely, on the front side 5 of the woven fabric 1.

In this case, according to Figure 5, where the thickness T the biopolymer layer 4 is T3, substantially all the dye is absorbed by the biopolymer layer 4; in other words, the dye does not substantially reach the surface (e.g. the front side 5) of the woven fabric 1, thus providing a treated fabric 100 having third regions 9 that are substantially not colored. Additionally, where the thickness T of the biopolymer layer 4 is T2, only part of the dye reaches the surface (e.g. the front side 5) of the woven fabric 1, thus providing a treated fabric 100 having second regions 8 that are slightly colored. Moreover, where the thickness T of the biopolymer layer 4 is T1, substantially all the dye reaches the surface (i.e. the front side 5) of the woven fabric 1, thus providing a treated fabric 100 having first regions 7, that are intensely colored.

As already mentioned, Figure 5, as Figure 4, has to be intended as a schematic representation of a treated fabric 100 according to the invention, because, the treated fabric 100 according to the invention presents numerous different color shades (i.e. a multi-shaded effect), due to the different penetration of the dye, through the thickness T of the biopolymer layer 4.

Figure 6, shows a perspective view of an exemplary embodiment of a treated fabric 100, having warp yarns 2 and weft yarns 3, and having a front side 5 and a back side 6, as obtainable by the process of the invention, i.e. after that at least part of the biopolymer layer 4 is removed from the composite fabric 10. Figure 6 shows an embodiment, wherein the biopolymer layer 4 has been completely removed from the composite fabric 10, e.g. from the front side 5 of the woven fabric 1, in step e. of the process of the invention.

Figure 6 shows an embodiment of the treated fabric 100 wherein second regions 8 cover the most of the front side 5 of the treated fabric 100. Treated fabric 100 presents first regions 7, which are intensely dyed, and third regions 9 which are substantially not dyed.

Therefore, a treated fabric 100 as shown in Figure 6 is substantially "slightly dyed", and presents intensely dyed regions (namely first regions 7), and substantially not-dyed regions (namely third regions 9), thus providing a "mixed" shade effect, i.e. a combination of a "dark on light" shade effect and a "light on dark" shade effect, e.g. a "mixed" worn out look.

For example, a treated fabric 100 according to Figure 6 can be obtained, when the biopolymer layer 4 (removed with step e. of the process of the invention) has a thickness T1 in correspondence of the first regions 7, a thickness T2>T1 in correspondence of second regions 8, and a thickness T3>T2>T1 in correspondence of third regions 9. For example, a biopolymer layer 4 having variable thickness T can be obtained by growing (i.e. producing) said biopolymer directly on the surface of the fabric, namely, on the front side 5 of the woven fabric 1. In this case, according to Figure 6, where the thickness is T3, the dye does not substantially reach the surface (i.e. the front side 5) of the woven fabric 1, thus providing a treated fabric 100 having third regions 9 that are substantially not colored. Where the thickness of the biopolymer layer 4 is T1, substantially all the dye reaches the woven fabric 1, thus providing a treated fabric 100 having first regions 7, that are intensely colored.

Additionally, where the thickness is T2, only part of the dye reaches the surface (i.e. the front side 5) of the woven fabric 1, thus providing a treated fabric 100 having second regions 8 that are slightly colored.

Figure 7, illustrates an exemplary embodiment of the treated fabric 100, having warp yarns 2 and weft yarns 3, and having a front side 5 and a back side 6, as obtainable by the process of the invention, i.e. after that at least part of the biopolymer layer 4 is removed from the composite fabric 10.

Figure 7 shows an embodiment, wherein the biopolymer layer 4 has been partially removed (i.e. not completely removed) from the composite fabric 10, e.g. from the front side 5 of the woven fabric 1, in step e. of the process of the invention.

Figure 7 shows an embodiment of the treated fabric 100 wherein residual bacterial biopolymer regions 4a are present on the front side 5 of the treated fabric 100. Said residual bacterial biopolymer regions 4a are dyed.

The embodiment of Figure 7 presents third regions 9, which cover the most of the front side 5 of the treated fabric 100; in other words, the most of the front surface of the treated fabric 100 is not dyed. Treated fabric 100 presents first regions 7, which are intensely dyed, and second regions 8 that are slightly colored (i.e., dyed with a lighter shade of color than the first regions 7).

The presence of the dyed residual bacterial biopolymer regions 4a on the treated fabric 100, provide a further "visual effect" which combines the peculiar color shade of the dyed biopolymer layer 4 with all the other shades of color on the treated fabric 100. Additionally, the presence of the residual bacterial biopolymer regions 4a provides the treated fabric 100 with a hand feel that is different from the hand feel of a fabric wherein the biopolymer layer 4 has been completely removed. With the varying of the amount of residual biopolymer layer 4 on the treated fabric 100 different hand touch effects can be obtained. Figure 8 shows an embodiment of the process of the invention, wherein the culture of biopolymer-producing microorganisms 200 is sprayed on an exemplary woven fabric 1 through a mesh wire 300. Woven fabric 1, has warp yarns 2 and weft yarns 3, and has a front side 5 and a back side 6. The woven fabric 1 represented in Figure 8 is not dyed. In the embodiment of the process of the invention illustrated in Figure 8, the culture of biopolymer-producing microorganisms 200 is sprayed on an exemplary woven fabric 1 through a mesh wire 300, by spraying means 201. The mesh wire 300 is placed between the woven fabric 1 and the spraying means 201, and has a mesh wire structure 301 defining mesh wire windows 302.

Spraying the culture of biopolymer-producing microorganisms 200 through the mesh wire 300, results in a non-homogeneous distribution of the biopolymer-producing microorganisms on the woven fabric 1. For example, a patterned distribution of the biopolymer-producing microorganisms can be obtained, thus providing the woven fabric 1, with regions that are contacted by the culture of biopolymer-producing microorganisms 200 and other regions that are not contacted by the sprayed culture of biopolymer-producing microorganisms 200. The mesh wire 300 may be made of any material; application of the culture may be made by screen-printing.

In other words, the mesh wire 300, that is placed on the front side 5 of the woven fabric 1, "hides" some regions of the woven fabric 1, i.e., the regions of the woven fabric 1 which lie under the mesh wire structure 301. The regions of the woven fabric 1 that are "hidden" by the mesh wire structure 301 are substantially not contacted by the culture of biopolymer-producing microorganisms 200 which is sprayed from the spraying means 201.

On the contrary, the sprayed culture of biopolymer-producing microorganisms 200 can reach the woven fabric 1 by passing through the mesh wire windows 302 of the mesh wire 300, which do not hide the woven fabric 1, and leave the portion of the woven fabric 1 in correspondence of the mesh wire windows 302 free to be contacted by the culture of biopolymer-producing microorganisms 200, sprayed by the spraying means 201.

As above mentioned, by culturing the biopolymer-producing microorganisms directly on the woven fabric 1, it is possible to grow (i.e. to produce) a biopolymer layer 4 directly on the woven fabric 1.

In exemplary embodiments, when the distribution of the biopolymer-producing microorganisms on the woven fabric 1 is a non-homogeneous distribution, a discontinuous (i.e. interrupted) biopolymer layer 4 can be obtained.

For example, as above mentioned, by spraying the culture of biopolymer-producing microorganisms 200 through the mesh wire 300 it is possible to obtain a woven fabric 1 having regions that are contacted by the culture of biopolymer-producing microorganisms 200 and other regions that are not contacted by the sprayed culture of biopolymer-producing microorganisms 200. In this case, a discontinuous (i.e. interrupted) biopolymer layer 4 can be obtained, thus providing a composite fabric 10 having a discontinuous (i.e. interrupted) biopolymer layer 4; in other words, a woven fabric 1 with regions that are covered by the biopolymer layer 4, and other regions which are not covered by the biopolymer layer 4 can be obtained.

Specifically, the regions of the woven fabric 1 contacted by the culture of biopolymer-producing microorganisms 200 are those regions of the woven fabric 1 which are in correspondence of the mesh wire windows 302 when the culture of biopolymer-producing microorganisms 200 is sprayed onto the woven fabric 1; such regions, after the culturing of the microorganism on the woven fabric 1, result to be regions of the composite fabric 10 that are provided with the biopolymer layer 4.

On the contrary, where the woven fabric 1 is hidden by the mesh wire structure 301 when the culture of biopolymer-producing microorganisms 200 is sprayed onto the woven fabric 1, the culture of biopolymer-producing microorganisms 200 does not substantially contact the woven fabric 1 and, therefore, the biopolymer layer 4 is not produced, thus providing regions of the composite fabric 10 that are not provided with the biopolymer layer 4. Preferably, the mesh wire 300 will be removed before dyeing once the layer, e.g., bacterial cellulose, is grown on the fabric, which is about 10 to 23 hours, e.g. 14-18 hours.

Figure 9 is a perspective view of a portion of an exemplary composite fabric 10, having a discontinuous biopolymer layer 4. The exemplary composite fabric 10 of Figure 9 is obtained by spraying a culture of biopolymer-producing microorganisms 200 through a mesh wire 300 on a woven fabric 1, and subsequently culturing the biopolymer-producing microorganisms directly on the woven fabric 1, without removing the mesh wire 300. The mesh wire 300 is preferably removed after the "growth" of the biopolymer layer 4 is completed to the desired degree, before the layer is removed at least in part from the fabric or the yarns.

The woven fabric 1 is thus coupled to a discontinuous biopolymer layer 4, providing a composite fabric 10. The exemplary embodiment of the composite fabric 10 of Figure 9, comprises a woven fabric 1 coupled to a discontinuous biopolymer layer 4, on its front side 5.

The back side 6 of the woven fabric 1 is also indicated in Figure 9. In this case, the back side 6 of the woven fabric 1 corresponds to the back side of the composite fabric 10.

In the embodiment of Figure 9, the biopolymer layer 4 is schematically represented as a discontinuous uniform layer. Namely, biopolymer layer 4 of Figure 9 is "discontinuous" because it covers the front side 5 of the woven fabric 1 with "interruptions", i.e. leaving regions that are not provided with the biopolymer layer 4. The biopolymer layer 4 of Figure 9 is "uniform", because it maintains the same thickness T over its entire extension.

In embodiments of the invention, the biopolymer layer 4 is a discontinuous non-uniform layer, i.e. it is an interrupted layer, and has a thickness T which is variable throughout the extension of the biopolymer layer 4.

Figure 9 shows an exemplary composite fabric 10 which is not dyed, i.e. which has not been subjected to a process of dyeing. Figure 10 is a perspective view of a portion of an exemplary composite fabric 10, having a discontinuous uniform biopolymer layer 4. In particular, Figure 10 shows the composite fabric 10 after dyeing. The exemplary embodiment of the composite fabric 10 of Figure 10, comprises a woven fabric 1 provided with a discontinuous uniform biopolymer layer 4, having thickness T, on its front side 5.

The back side 6 of the woven fabric 1 is also indicated in Figure 10. In this case, the back side 6 of the woven fabric 1 corresponds to the back side of the composite fabric 10.

According to the embodiment of Figure 10, the biopolymer layer 4 is a discontinuous biopolymer layer 4, and the regions of the woven fabric 1 which are not coupled with (namely "not covered by") the biopolymer layer 4 are dyed, as well as the biopolymer layer 4.

Figure 11 shows a perspective views of an exemplary embodiment of a treated fabric 100 as obtainable by the process of the invention, i.e. after that at least part of the biopolymer layer 4 is removed from the composite fabric 10. Figure 11 shows a treated fabric 100, having warp yarns 2 and weft yarns 3 and having a front side 5 and a back side 6.

Figure 11 shows an embodiment wherein the biopolymer layer 4 has been completely removed from the woven fabric 1, and that is obtainable when the biopolymer layer 4 of the composite fabric 10 is a discontinuous layer, such as, for example, in the composite fabric 10 illustrated in Figure 10 and Figure 9.

The treated fabric 100 of Figure 11 presents, on its front side 5, first regions 7 that are intensely colored, second regions 8 that are slightly colored (i.e., dyed with a lighter shade of color than the first regions 7), and third regions 9 that are substantially not colored, i.e. not dyed.

Figure 11 shows an embodiment of the treated fabric 100 wherein first regions 7 correspond to those regions that were not coupled with the biopolymer layer 4, i.e. those regions where the thickness T of the biopolymer layer 4 was zero. The treated fabric 100 of Figure 11 further presents second regions 8 which are colored with a lighter shade of dye than the first regions 7, and third regions 9 which are substantially not dyed.

Third regions 9 are obtained, for example, when the dye that is applied to the composite fabric 10 is completely absorbed by the biopolymer layer 4 and, therefore, does not reach the woven fabric 1, which remains undyed.

Second regions 8 are obtained, for example, when part of the dye that is applied to the composite fabric 10 reaches the woven fabric 1, thus providing the treated fabric 100 with second regions 8 which are colored with a lighter shade of dye than the first regions 7, when the biopolymer layer 4 is removed. First regions 7 are obtained, for example, when the majority of the dye that is applied to the composite fabric 10 reaches the woven fabric 1.

Figure 11 is a schematic representation of a treated fabric 100 according to the invention; in fact, the treated fabric 100 of the invention have a shaded appearance, i.e. the treated fabric 100 presents numerous different color shades, due to the different penetration of the dye, throughout the biopolymer layer 4, namely through the thickness T of the biopolymer layer 4.

As above discussed, this is particularly true in the embodiments of the invention, where the biopolymer layer 4 has a thickness T that is not the same throughout the extension of the biopolymer layer 4, i.e. thickness T can assume different values (e.g. T1, T2, T3) in different regions of the biopolymer layer 4, i.e. the biopolymer layer 4 is non-uniform.

The number of the shades of color is further increased in those embodiments wherein the biopolymer layer 4 is discontinuous. In fact, the dye uptake of the composite fabric 10 is substantially determined by the thickness T of the biopolymer layer 4. In particular, it has been observed that, the higher is the thickness T, the higher is the dye uptake. In other words, when a composite fabric 10 presents a biopolymer layer 4 having variable thickness T, different amounts of dye reach the surface (i.e., for example, the front side 5) of the woven fabric 1.

For example, if the thickness T of the biopolymer layer 4 is high, a little, or none, dye reaches the surface (i.e., for example, the front side 5) of the woven fabric 1, thus providing the treated fabric 100 with second regions 8 that are slightly colored and/or third regions 9 that are substantially not colored, i.e. not dyed.

On the contrary, for example, if the thickness T of the biopolymer layer 4 is low, or the biopolymer layer 4 is absent (e.g. when the biopolymer layer 4 is discontinuous) a great amount of dye reaches the surface (i.e., for example, the front side 5) of the woven fabric 1, thus providing the treated fabric 100 with first regions 7, that are intensely colored.

### Examples

The following examples will be better illustrate an exemplary process for the production for the production of a treated fabric according to the invention. The following examples are to be interpreted as merely illustrative and they do not limit the scope of the invention.

### Example 1

25 ml of a culture of *Gluconacetobacter hansenii* having a concentration of 2x10⁴cells/ml, is sprayed culture on a the front side of a sample woven fabric according to the invention. The culture used is a culture of *Gluconacetobacter hansenii,* in in Hestrin-Schramm (HS) medium containing 2% (w/v) glucose, 0,5 %(w/v) peptone, 0,5% (w/v) yeast extract, 0,27% (w/v) Na2HPO4 and 1,15g/L citric acid.

Illustrative examples of woven fabrics according to the invention, which were used according to the present "Examples" are the following:

### 1. "Rigid"- 12oz 100% cotton:

Warp yarns are Ne 7/1 - 10/1
Weft yarns are Ne 8/1 - 10/1
Warp density of the fabric is 25-28 threads/cm
Weft density of the fabric is 17-20 picks/cm
The weight of the woven fabric is 640-670 g/m
The front side of the woven fabric has a surface density of 407-423 g/m² Materials that can be used for the woven fabric, in particular for warp yarns, are cotton, cotton and other staple fibers blend, or staple fibers apart from cotton (Cotton/Tencel, Cotton/Modal, Cotton/PES, Cotton/Bamboo, 100%PES, 100% Tencel, Modal or Tencel/Modal blends).

### 2. "Comfort" - 12oz cotton/elastane (18%-25% elasticity)

Warp yarns are Ne 7/1 - 10/1
Weft yarns are Ne 10/1 - 12/1
Warp density of the fabric is 27-31 threads/cm
Weft density of the fabric is 17-21 picks/cm
The weight of the woven fabric is 500-550 g/m
The front side of the woven fabric has a surface density of 407-423 g/m² Materials that can be used for the woven fabric, in particular for warp yarns, are cotton, cotton and other staple fibers blend, or staple fibers apart from cotton (Cotton/Tencel, Cotton/Modal, Cotton/PES, Cotton/Bamboo, 100%PES, 100% Tencel, Modal or Tencel/Modal blends).

### 3. "Super stretch" - 12oz cotton/elastane (40%-65% elasticity)

Warp yarns are Ne 9/1 - 12/1
Weft yarns are Ne 15/1 - 18/1
Warp density of the fabric is 29-32 threads/cm
Weft density of the fabric is 20-24 picks/cm
The weight of the woven fabric is 464-490 g/m
The front side of the woven fabric has a surface density of 407-423 g/m² Materials that can be used for the woven fabric, in particular for warp yarns, are cotton, cotton and other staple fibers blend, or staple fibers apart from cotton (Cotton/Tencel, Cotton/Modal, Cotton/PES, Cotton/Bamboo, 100%PES, 100% Tencel, Modal or Tencel/Modal blends).

### Example 2

After the application (spraying) of the bacterial culture of Example 1 on the woven fabric, the woven fabric is incubated for 16 hours, at temperature 28 °C. After 16 hours, at temperature 28 °C, a layer of bacterial cellulose having a thickness ranging from 0,5mm to 1 mm, with an average value of 0,75 mm is obtained on the front side of the woven fabric, i.e. a composite fabric is obtained.

### Example 3

After the bacterial cellulose layer growth is completed, the composite fabric obtained in Example 2 is washed with 0,1M NaOH at 80°C temperature to remove the residual bacteria and all the impurities coming from the growth medium including the bacteria, and in NaOCl, for 20 minutes to remove the residual bacteria from the composite fabric.

After the removal of residual bacteria and all the impurities coming from the growth medium including the bacteria, the composite fabric is print-dyed, with a dye selected from indigo, pigments, reactive, sulphur dyes, preferably with indigo on its front side, i.e. on the side wherein the bacterial cellulose layer is present.

Alternatively, the composite fabric may be VAT dyed with conventional indigo dyeing (i.e. on both sides of the fabric).

### Example 4

The dyed composite fabric obtained in Example 3 is finished through one or more finishing techniques.

For example the dyed composite obtained in Example 3 may be rinsed with water 20 minutes at 40°C. Additionally or alternatively, the dyed composite fabric obtained in Example 3 may be or stone washed (i.e. washed in the presence of pumice stone) 20 minutes at 40°C, followed by enzyme wash for 10 minutes at 50°C to remove small hair (pilling) created by the stone wash. Additionally or alternatively, the dyed composite obtained in Example 3 may undergo stone bleaching, for 20 minutes at 40°C. Additionally or alternatively, the dyed composite fabric obtained in Example 3 may undergo laser treatments. One or more of the above mentioned techniques are used to remove the bacterial cellulose layer, thus obtaining a treated fabric according to the invention.

## Claims

1. A process for producing a treated fabric (100), comprising the following steps:
a. Providing at least one plurality of warp yarns (2) and at least one plurality of weft yarns (3);
b. Weaving said at least one plurality of warp yarns (2) with said at least one plurality of weft yarns (3) to provide a woven fabric (1), having a front side (5) and a back side (6);
c. Providing at least a layer (4) of at least one biopolymer which is produced by a microorganism on said yarns (2; 3) or on at least part of at least one side (5; 6) of said woven fabric (1) to provide a composite fabric (10);
**characterized in that** said process comprises the steps of
d. Dyeing at least part of said composite fabric (10), whereby at least part of the fabric yarns (2; 3) are dyed together with said biopolymer layer (4);
e. Removing at least part of said layer (4) of biopolymer from said composite fabric (10) to obtain a treated fabric (100);
wherein said step c. is carried out after step b. by producing said biopolymer layer (4) on the woven fabric (1) or before step b. by producing said biopolymer layer (4) on said yarns before weaving said fabric,
wherein said step c. is carried out by contacting at least part of said woven fabric (1) or at least part of said yarns (2; 3) with a culture of microorganisms (200) producing a biopolymer, and culturing said biopolymer-producing microorganisms, to provide at least part of said woven fabric (1) or at least part of said yarns (2; 3) with a biopolymer layer (4).

2. A process according to claim 1, wherein the thickness (T) of said at least one layer (4) of biopolymer is non-uniform throughout the extension of said biopolymer layer (4).

3. A process according to claim 1 or 2, wherein at least part of said at least one biopolymer layer (4) is a discontinuous layer.

4. A process according to any previous claim, wherein said layer (4) of biopolymer produced by a microorganism is selected from a sugar-based biopolymer, preferably cellulose produced by bacteria and/or algae, and an amino acid-based biopolymer, preferably collagen produced by bacteria, or a mixture thereof.

5. A process according to claim 1, wherein said culture of biopolymer-producing microorganisms (200) is sprayed on at least part of said woven fabric (1), preferably on at least part of the front side (5) of said woven fabric (1).

6. A process according to claim 5, wherein said culture of biopolymer-producing microorganisms (200) is sprayed on at least part of said woven fabric (1) through a mesh wire (300).

7. A process according to claim 1, at least part of said woven fabric (1) or at least part of said yarns (2; 3) is contacted with a culture of microorganisms (200) producing a biopolymer by dipping said at least part of said woven fabric (1) or at least part of said yarns (2; 3) into said culture of biopolymer-producing microorganisms.

8. A process according anyone of claims 1 to 7, wherein said biopolymer-producing microorganisms are selected from biopolymer-producing bacteria, biopolymer-producing algae, and mixtures thereof, wherein biopolymer-producing bacteria are preferably selected from *Gluconacetobacter, Aerobacter, Acetobacter, Achromobacter, Agrobacterium, Azotobacter, Salmonella, Alcaligenes, Pseudomonas, Rhizobium, Sarcina and Streptoccoccus, Bacillus* genus, and mixtures thereof, and wherein biopolymer-producing algae are preferably selected from *Phaeophyta, Rhodophyta* and *Chrysophyta,* and mixture thereof.

9. A process according to any previous claim, wherein said woven fabric (1) comprises a plurality of warp yarns (2) and/or a plurality of weft yarns (3) that forms an additional layer of said woven fabric (1) in the form of loop portions on at least one of the sides (5; 6) of said woven fabric (1), wherein at least part of said additional layer is included into said biopolymer layer (4).

10. A process according to any previous claim, wherein, said warp yarns (2) and/or said weft yarns (3) are selected from natural yarns, synthetic yarns and mixed yarns, wherein said natural yarns comprise natural fibers selected from cotton, wool, flax, kenaf, ramie, hemp, and mixtures thereof, wherein said synthetic yarns comprise synthetic fibers selected from polyester, rayon, nylon, lycra and mixtures thereof, and wherein mixed yarns comprise both natural fibers and synthetic fibers.

11. A process according to any previous claim, wherein said woven fabric (1) is a denim fabric.

12. A process according to any previous claim, wherein said step d. is selected from print-dyeing, indigo dyeing, dipping said composite fabric into a dye bath, wherein preferably the dye is indigo dye.

13. A process according to any previous claim, wherein said step e. is carried out by laundry washing and/or abrading at least part of said at least one biopolymer layer (4) from said composite fabric (10).

## Patentansprüche

1. Verfahren zur Herstellung eines behandelten Gewebes (100), umfassend die folgenden Schritte:
a. Bereitstellen von mindestens einer Vielzahl von Kettfäden (2) und mindestens einer Vielzahl von Schussfäden (3);
b. Weben der mindestens einen Vielzahl von Kettfäden (2) mit der mindestens einen Vielzahl von Schussfäden (3), um ein Gewebe (1) bereitzustellen, das eine Vorderseite (5) und eine Rückseite (6) aufweist;
c. Bereitstellen von mindestens einer Schicht (4) aus mindestens einem durch einen Mikroorganismus hergestellten Biopolymer auf den Garnen (2; 3) oder auf mindestens einem Teil von mindestens einer Seite (5; 6) des Gewebes (1), um ein Verbundgewebe (10) bereitzustellen;
**dadurch gekennzeichnet, dass** das Verfahren die folgenden Schritte umfasst
d. Färben von mindestens einem Teil des Verbundgewebes (10), wobei mindestens ein Teil der Gewebegarne (2; 3) zusammen mit der Biopolymerschicht (4) gefärbt wird;
e. Entfernen von mindestens einem Teil der Schicht (4) von Biopolymer von dem Verbundgewebe (10), um ein behandeltes Gewebe (100) zu erhalten;
wobei der Schritt c. nach dem Schritt b. durch Herstellen der Biopolymerschicht (4) auf dem Gewebe (1) oder vor Schritt b. durch Herstellen der Biopolymerschicht (4) auf den Garnen vor dem Weben des Gewebes ausgeführt wird;
wobei der Schritt c. durchgeführt wird durch Inkontaktbringen mindestens eines Teils des Gewebes (1) oder mindestens eines Teils der Garne (2; 3) mit einer Kultur von Mikroorganismen (200), die ein Biopolymer herstellen, und Kultivieren der Biopolymer herstellenden Mikroorganismen, um mindestens einen Teil des Gewebes (1) oder mindestens einen Teil der Garne (2; 3) mit einer Biopolymerschicht (4) bereitzustellen.

2. Verfahren nach Anspruch 1, wobei die Dicke (T) der mindestens einen Schicht (4) des Biopolymers über die gesamte Ausdehnung der Biopolymerschicht (4) ungleichmäßig ist.

3. Verfahren nach Anspruch 1 oder 2, wobei mindestens ein Teil der mindestens einen Biopolymerschicht (4) eine diskontinuierliche Schicht ist.

4. Verfahren nach einem der vorherigen Ansprüche, wobei die Schicht (4) des durch einen Mikroorganismus hergestellten Biopolymers ausgewählt ist aus einem Biopolymer auf Zuckerbasis, vorzugsweise durch Bakterien und/oder Algen hergestellte Cellulose, und einem Biopolymer auf Aminosäurebasis, vorzugsweise durch Bakterien hergestelltes Kollagen, oder einer Mischung davon.

5. Verfahren nach Anspruch 1, wobei die Kultur von Biopolymer herstellenden Mikroorganismen (200) auf mindestens einen Teil des Gewebes (1) gesprüht wird, vorzugsweise auf mindestens einen Teil der Vorderseite (5) des Gewebes (1).

6. Verfahren nach Anspruch 5, wobei die Kultur von Biopolymer herstellenden Mikroorganismen (200) auf mindestens einen Teil des Gewebes (1) durch ein Drahtgeflecht (300) gesprüht wird.

7. Verfahren nach Anspruch 1, bei dem mindestens ein Teil des Gewebes (1) oder mindestens ein Teil der Garne (2; 3) mit einer Kultur von Biopolymer herstellenden Mikroorganismen (200) durch Eintauchen des mindestens einen Teils des Gewebes (1) oder des mindestens einen Teils der Garne (2; 3) in die Kultur von Biopolymer herstellenden Mikroorganismen in Kontakt gebracht wird.

8. Verfahren nach einem der Ansprüche 1 bis 7, wobei die Biopolymer herstellenden Mikroorganismen aus Biopolymer herstellenden Bakterien, Biopolymer herstellenden Algen und einer Mischungen davon ausgewählt sind, wobei die Biopolymer herstellenden Bakterien vorzugsweise aus *Gluconacetobacter, Aerobacter, Acetobacter, Achromobacter, Agrobacterium, Azotobacter, Salmonella, Alcaligenes, Pseudomonas, Rhizobium, Sarcina* und *Streptoccoccus,* Bacillus-Gattung und Mischungen davon ausgewählt sind, wobei die Biopolymer herstellenden Algen vorzugsweise aus *Phaeophyta, Rhodophyta* und *Chrysophyta* und einer Mischung davon ausgewählt sind.

9. Verfahren nach einem der vorherigen Ansprüche, wobei das Gewebe (1) eine Vielzahl von Kettfäden (2) und/oder eine Vielzahl von Schussfäden (3) umfasst, die eine zusätzliche Schicht des Gewebes (1) in der Form von Schlaufenabschnitten auf mindestens einer der Seiten (5; 6) des Gewebes (1) bilden, wobei mindestens ein Teil der zusätzlichen Schicht in der Biopolymerschicht (4) enthalten ist.

10. Verfahren nach einem der vorherigen Ansprüche, wobei die Kettfäden (2) und/oder die Schussfäden (3) aus Naturgarnen, synthetischen Garnen und Mischgarnen ausgewählt sind, wobei die Naturgarne Naturfasern umfassen, die aus Baumwolle, Wolle, Flachs, Kenaf, Ramie, Hanf und Mischungen davon ausgewählt sind, wobei die synthetischen Garne synthetische Fasern umfassen, die aus Polyester, Rayon, Nylon, Lycra und Mischungen davon ausgewählt sind, und wobei die Mischgarne sowohl natürliche Fasern als auch synthetische Fasern umfassen.

11. Verfahren nach einem der vorherigen Ansprüche, wobei das Gewebe (1) ein Denimgewebe ist.

12. Verfahren nach einem der vorherigen Ansprüche, wobei der Schritt d. aus Druckfärben, Indigofärben, Eintauchen des Verbundgewebes in ein Färbebad ausgewählt ist, wobei der Farbstoff vorzugsweise Indigofarbstoff ist.

13. Verfahren nach einem der vorherigen Ansprüche, wobei der Schritt e. durch Waschen und/oder Abschleifen mindestens eines Teils der mindestens einen Biopolymerschicht (4) aus dem Verbundgewebe (10) durchgeführt wird.

## Revendications

1. Procédé pour produire un tissu traité (100) comprenant les étapes suivantes consistant à :
a. fournir au moins une pluralité de fils de chaîne (2) et au moins une pluralité de fils de trame (3) ;
b. tisser ladite au moins une pluralité de fils de chaîne (2) avec ladite au moins une pluralité de fils de trame (3) pour fournir un tissu tissé (1) ayant un côté avant (5) et un côté arrière (6) ;
c. fournir au moins une couche (4) d'au moins un biopolymère qui est produit par un microorganisme sur lesdits fils (2 ; 3) ou sur au moins une partie d'au moins un côté (5 ; 6) dudit tissu tissé (1) pour fournir un tissu composite (10) ;
**caractérisé en ce que** ledit procédé comprend les étapes consistant à
d. teindre au moins une partie dudit tissu composite (10), grâce à quoi au moins une partie des fils de tissu (2 ; 3) sont teintés conjointement avec ladite couche de biopolymère (4) ;
e. enlever au moins une partie de ladite couche (4) de biopolymère dudit tissu composite (10) pour obtenir un tissu traité (100) :
dans lequel ladite étape c. est effectuée après l'étape b. en produisant ladite couche de biopolymère (4) sur le tissu tissé (1) ou avant l'étape b. en produisant ladite couche de biopolymère (4) sur lesdits fils avant de tisser ledit tissu,
dans lequel ladite étape c. est effectuée en mettant en contact au moins une partie dudit tissu tissé (1) ou au moins une partie desdits fils (2 ; 3) avec une culture de microorganismes (200) produisant un biopolymère, et en cultivant lesdits microorganismes produisant un biopolymère pour fournir au moins une partie dudit tissu tissé (1) ou au moins une partie desdits fils (2 ; 3) avec une couche de biopolymère (4).

2. Procédé selon la revendication 1, dans lequel l'épaisseur (T) de ladite au moins une couche (4) de biopolymère est non uniforme tout au long de l'extension de ladite couche de biopolymère (4).

3. Procédé selon la revendication 1 ou 2, dans lequel au moins une partie de ladite au moins une couche de biopolymère (4) est une couche discontinue.

4. Procédé selon l'une quelconque des revendications précédentes, dans lequel ladite couche (4) de biopolymère produit par un microorganisme est sélectionnée parmi un biopolymère à base de sucre, de préférence de la cellulose produite par des bactéries et/ou des algues, et un biopolymère à base d'acide aminé, de préférence du collagène produit par des bactéries, ou un mélange de ceux-ci.

5. Procédé selon la revendication 1, dans lequel ladite culture de microorganismes produisant un biopolymère (200) est pulvérisée sur au moins une partie dudit tissu tissé (1), de préférence sur au moins une partie du côté avant (5) dudit tissu tissé (1).

6. Procédé selon la revendication 5, dans lequel ladite culture de microorganismes produisant un biopolymère (200) est pulvérisée sur au moins une partie dudit tissu tissé (1) au moyen d'un fil de maille (300).

7. Procédé selon la revendication 1, au moins une partie dudit tissu tissé (1) ou au moins une partie desdits fils (2 ; 3) est mise en contact avec une culture de microorganismes (200) produisant un biopolymère en plongeant au moins une partie dudit tissu tissé (1) ou au moins une partie desdits fils (2 ; 3) dans ladite culture de microorganismes produisant un biopolymère.

8. Procédé selon l'une quelconque des revendications 1 à 7, dans lequel lesdits microorganismes produisant un biopolymère sont sélectionnés parmi des bactéries produisant un biopolymère, des algues produisant un biopolymère et des mélanges de celles-ci, dans lequel les bactéries produisant un biopolymère sont, de préférence, sélectionnées parmi *Gluconacetobacter, Aerobacter, Acetobacter, Achromobacter, Agrobacterium, Azotobacter, Salmonella, Alcaligenes, Pseudomonas, Rhizobium, Sarcina* et *Streptoccoccus,* le genre *Bacillus,* et des mélanges de ceux-ci, et dans lequel les algues produisant un biopolymère sont, de préférence, sélectionnées parmi *Phaeophyta, Rhodophyta* et *Chrysophyta* et des mélanges de ceux-ci.

9. Procédé selon l'une quelconque des revendications précédentes, dans lequel ledit tissu tissé (1) comprend une pluralité de fils de chaîne (2) et/ou une pluralité de fils de trame (3) qui forment une couche supplémentaire dudit tissu tissé (1) sous la forme de parties de boucle sur au moins l'un des côtés (5 ; 6) dudit tissu tissé (1), dans lequel au moins une partie de ladite couche supplémentaire est incluse dans ladite couche de biopolymère (4).

10. Procédé selon l'une quelconque des revendications précédentes, dans lequel lesdits fils de chaîne (2) et/ou lesdits fils de trame (3) sont sélectionnés parmi des fils naturels, des fils synthétiques et des fils mixtes, dans lequel lesdits fils naturels comprennent des fibres naturelles sélectionnées parmi le coton, la laine, le lin, le chanvre de Gambo, la ramie, le chanvre, et des mélanges de ceux-ci, dans lequel lesdits fils synthétiques comprennent des fibres synthétiques sélectionnées parmi le polyester, la rayonne, le nylon, l'élasthanne et des mélanges de ceux-ci et dans lequel des fils mixtes comprennent à la fois des fibres naturelles et des fibres synthétiques.

11. Procédé selon l'une quelconque des revendications précédentes, dans lequel ledit tissu tissé (1) est un tissu denim.

12. Procédé selon l'une quelconque des revendications précédentes, dans lequel l'étape d. est sélectionnée parmi la teinture par impression, la teinture à l'indigo, l'immersion dudit tissu composite dans un bain de teinture, dans lequel, de préférence, le colorant est le colorant indigo.

13. Procédé selon l'une quelconque des revendications précédentes, dans lequel ladite étape e. est réalisée en lavant le linge et/ou en usant par abrasion au moins une partie de ladite au moins une couche de biopolymère (4) dudit tissu composite (10).
